

## UNITED STATES PATENT OFFICE

2,643,186

## PROCESS OF FORMING ARTIFICIAL BOARD

Gordon E. Tower, Corvallis, Oreg., assignor to  
 Chapman Forest Utilization, Inc., Corvallis,  
 Oreg., a corporation of Oregon

No Drawing. Application April 10, 1948,  
 Serial No. 20,353

2 Claims. (Cl. 92—21)

1

My present invention relates to the fibreboard art in that the principal object of the present invention is to provide a novel method for forming a novel fibreboard, the invention, however, being applicable to the formation of other fibre products having boardlike characteristics, such as molded panels, plates, insulating members and other articles of a similar nature.

The principal object of the present invention is to provide a board which will have increased strength, modulus of rupture, resistance to moisture absorption, resistance to swelling or warping, and resistance to the effects of acids, alkalies, steam, heat, dry rot and fungus or to destruction by termites and rodents.

It is well known in the art that boards or boardlike products may be created by reducing wood or woody substances such as cornstalks, straw, leaves, grass, hemp, esparto grass, flax, papyrus, ramie and other fibrous substances to fibres, forming a water slurry of the fibres, adding thereto a solution of a phenol-formaldehyde resin, straining the water from the fibres to form a mat, and compressing the fibre mats while heating them to convert the resin and the natural lignins or other resinous substances present in and among the fibres, to an infusible, insoluble state. Examples of such processes are disclosed, for example, in the patents to Baekeland 1,160,362 and 1,160,365, Cheetham 1,776,885 and Novotny et al. 1,616,062. Various means are known for disintegrating wood or woody substances into fibres such as by grinding or abrading chips of wood, by soaking wood chips in water, or subjecting them to steam, until they disintegrate into fibrous bundles, by chemical digestion, or by the well known explosion process disclosed in the patent to Mason 1,578,609. Various means are known whereby fibre slurries may be made into boards, such as wholly or partially disclosed in the patents to Mason 1,603,503, 1,603,504, 1,603,505 and 1,603,506; Vogt 1,718,011; Vogt et al. 1,718,012; Streeter 1,763,910; and Mason 1,767,539. It is the collective teaching of the art as identified above that a board or boardlike article having a density ranging from 0.5 to 1.0 or higher and composed of fibres bound by C-stage phenolic resins or the natural resins of the wood fibres, or by both, may be formed. In the process of consolidating the boards or other articles wet mats of fibres are preferably heated between rolls or platens at temperatures higher than the boiling point of water and pressures of at least several times atmospheric pressure for various periods of time and with various alterations of the tem-

2

perature or pressure during the time the articles are being pressed. During the drying operation the water which is present in the wet mat of fibres is either squeezed from the article as freely running hot water or escapes therefrom as steam. An object of several of the foregoing patents is to provide ways and means whereby migration of the resin either to or from the surfaces of the sheets, and migration of other substances present in or among the fibres such as wood sugars which char upon contact with the hot platens, is diminished. An object of the present invention is to provide a method whereby the resin added to a fibre slurry is retained during the hot pressing operation in intimate contact with all of the fibre, without migration thereof to surface or edge areas under the force of escaping steam and running hot water under pressure.

In the foregoing patents the step of adding a phenolic resin in comminuted state or in solution is disclosed, and the precipitation of the phenolic resin after thorough mixture with the slurry is also disclosed. In accordance with my improvement a time lag is permitted between addition of the resin solution to the fibres and the precipitation thereof, such time lag being of sufficient length to establish a firm bond between the fibres and the resin molecules. The bond thus established appears to be partly in the nature of adsorption, a surface phenomenon whereby molecules of the resin attach themselves to the surfaces of the fibres, and absorption, an osmotic action wherein the molecules of the resin intermingle with the molecules of the fibres, perhaps accompanied by a chemical linkage of the phenolic material with the cellulosic substance forming the fibres, or with other natural substances found with wood fibres such as lignins and hemicellulose.

Adsorption in itself takes place rapidly. However, it requires time to manipulate the resin molecules into position to be adsorbed due to the irregular surfaces of the fibres and the cell wall openings. If the time of mixing is short only those resin molecules which have had the opportunity to be adsorbed by the outside surfaces of the fibres, and particles physically held by the fibre web, are retained, with the result that a large proportion of the precipitated resin is freely suspended in the water slurry and drains off from the fibres in the white water resulting from the screening process of forming a wet mat of tangled fibres. In accordance with my invention, I permit sufficient time for the processes of diffusion, absorption and adsorption of the resin

molecules to take place throughout the fibre slurry. Upon precipitation those molecules on the surface of the fibre act as nuclei about which resin particles form from resin in the water solution surrounding the fibres. Whatever the exact phenomena might be, I have discovered that permitting the resin to remain in solution for a substantial period of time with the fibre particles, such as approximately one-half hour, results in the retention of eighty to ninety per cent of the resin by the fibres, whereas immediate precipitation results in retention of a lesser proportion, such as approximately fifty to sixty percent.

The rate of diffusion into and hence the retention of the resin by the wood fibres appears to be affected by the sizes of various openings in the individual fibres such as pits, fibre cavities and cell wall capillaries, into which the resin diffuses.

While any of several phenolic resins may be utilized with good results in my process, I have also determined that a resin polymer of large molecular size is most desirable, apparently because the attraction or bond between the fibres and resin is most advantageous if the resin molecules remain largely upon or close to the surfaces of the fibres. Some resins of smaller molecular size penetrate deeply into the interiors of the fibres and thus fail to bind adjacent fibres together when converted into C-stage. I have determined that many of the commercially available phenolic resins may be utilized to good advantage, but I prefer a phenol-formaldehyde resin, such resin being of the type which is water-soluble and alkaline in nature. I prefer to form an alkaline solution of a water-soluble phenolic condensation product in the B-stage or in the incipient C-stage as expressed by D. V. Redfern of the American Marietta Chemical Company. In accordance with Mr. Redfern's discoveries the reaction of a mixture of phenol and formaldehyde may be advanced to form a resin almost to the end of the B-stage by the controlled stepwise addition of sodium hydroxide as a catalyst and solubilizer. It is not my intention to relate herein the exact details of Redfern's process, it being sufficient to state that the product obtained from his process is an alkaline, water-soluble, phenol-formaldehyde resin in incipient C-stage having a very large molecular structure. This resin has the additional advantage of being recapturable from precipitation a number of times. That is, after the alkaline solution has been precipitated the resin may be reused by restoring its alkalinity a number of times, whereas some resin products which have been once precipitated form an end product, all of which cannot be returned to solution by alkalinizing the water holding the precipitate. It is immaterial to the present invention to describe the method of manufacturing Redfern's resin, such method being disclosed and claimed in the copending application of D. V. Redfern, Serial No. 722,016, filed September 3, 1947, now Reissue Patent 23,347, reissued March 20, 1951. Such a resin is herein referred to as an intermediate condensation product of the phenol-formaldehyde type in incipient C-stage resulting from controlled step reactions in the presence of an alkaline catalyst such as sodium hydroxide.

I have discovered that delayed addition of acid or acidic salts to acidify or substantially neutralize the alkaline mixture of fibres and resin in a slurry to establish retention of the resin by

the fibres accomplishes results comparable to results which have heretofore only been achieved by hydrolyzing or otherwise treating cellulosic fibres until the fibre has been converted to viscose or a purified cellulose as distinguished from a ligno-cellulose type of material. The hydrolyzing action converts raw wood fibre, as distinguished from chemically produced fibres, apparently both chemically and mechanically, to a slimy, viscous substance having the individual fibres more or less reduced to a pulpy or gelatinous state, each fibre having far less mechanical strength than the original fibre. By my process I am able to achieve firmly bonded fibrous products in which the individual fibres remain as naturally created with the exception of some swelling due to absorption of water. This is accomplished without expensive machinery such as beaters and jordans, and without the loss of time required for producing hydrolyzed cellulose. In my process I am able to take green or dry wood, mechanically convert it to individual fibres or small bundles of fibres by grinding or crushing machines, or by mechanical defibrizers having teeth which gouge slivers from the lengths of wood stock, or other suitable process, and form a slurry thereof which may be immediately started through the board-forming process. No digestion or other chemical reaction is required, but digested pulp may be used if desired.

The slurry of fibres is formed by adding water, preferably including white water drained from previously formed mats or resin-bearing fibres so as to recapture the particles of precipitated resin which have escaped from the fibres of the previously formed mats, such precipitated resins being mechanically retained by the straining action of the fibres being formed into mats, or redissolved when an alkaline solution of resin is added to the slurry. This redissolving of the resin is more readily accomplished and may be repeated a number of times with a resin such as formed by the Redfern process, but other phenolic resins may be utilized with some degree of success since the precipitate which will not redissolve is largely recaptured by the straining action of the fibres, especially when the fibres have become somewhat sticky due to the adherence thereto of resin in accordance with my process.

The fibre slurry is preferably formed with a consistency of about one to three per cent for ease of pumping and is pumped through refiners which assure the elimination of all large bundles of fibres by separating them into individual fibres or fibre bundles of small dimensions. From the refiners the slurry is pumped into a precipitating vat preferably having agitating means therein to assure thorough mixing of the resin solution which is added at this point. The resin solution is preferably added as an alkaline solution, the amount of resin being varied in accordance with the hardness or strength or other qualities desired in the finished product. Resin in the proportion of two per cent resin solids to fibre based on the dry weight of the fibre will give a satisfactory hardboard suitable for many purposes, while as high as forty per cent resin may be incorporated to form a non-porous board or article. The amount of resin can be adjusted to give properties to the product in accordance with the intended use of the finished product, but three and one-half per cent is a suitable amount for most purposes.

The resin is allowed to remain in solution for a

sufficient period of time to establish sorption thereof. By the word "sorption" I mean to include the phenomena of adsorption, absorption and diffusion. Although some of the resin is immediately retained, I have found that approximately one-half hour is required as the minimum time for the retention of over ninety per cent of the resin. The amount of retention may be expressed against the time factor as a parabolic curve, for example, less than fifty per cent being retained in the first five minutes, about seventy-five per cent in the first twenty minutes and about ninety per cent being retained in thirty minutes. If the resin remains in solution for a longer length of time the curve flattens out toward infinity with the additional advantage gained in several hours' time being slight. The practical application of my process therefore comprises the step of allowing the resin to remain in solution in the range of twenty minutes to one hour. After sorption of the resin is accomplished, precipitation of the resin is achieved by acidifying or substantially neutralizing the alkaline mixture. Sulfuric acid, hydrochloric acid or acidic salts such as alum may be used, but for reasons of economy a ten per cent solution of sulfuric acid appears best. The pH of the fibre resin slurry may be between 7.5 and 10.5, and sufficient acid or acidic salt is used to achieve a final pH of about 5.5. The final pH is not critical and may be in the range of 4.5 to 6.0. Immediately upon establishing thorough mixing of the acidifying agent the slurry may be strained to form a wet mat of entangled fibres having the resin bound thereto, at least partially by sorption, which may then be consolidated under heat and pressure to form the desired end product. By varying the temperature and pressure, as well as the thickness of the article being formed, the density of the final product may be varied as desired. For example, boards may be formed with densities ranging from 0.5 to 1.4 in thicknesses of one-sixteenth to one inch or greater.

After the formation of the boards or other articles their humidity is adjusted by conditioning them for a sufficient period of time in a humid atmosphere until they reach a moisture content of approximately seven per cent.

Boards made in accordance with my process have improved characteristics, such as the modulus of rupture in static bending being 6500 p. s. i. for four per cent resin to dry weight of fibre when using Redfern resin, and 5100 p. s. i. to 5800 p. s. i. when using several other phenolic resins, as compared with 2800 p. s. i. for a board incorporating no artificial resin. Samples immersed in water for eight days at 70° F. will swell in thickness approximately thirty per cent when incorporating four per cent of any of the resins as compared with approximately seventy-five per cent for a board having no resin; and will swell laterally approximately 0.15 per cent when incorporating four per cent resin as compared to approximately 0.7 per cent for a board having no resin. The above figures were taken from samples of board formed in identical manner in all cases except for the resin variation. The boards measured approximately 0.21 inch in thickness and had a specific gravity of approximately 0.95.

In a variation of my process, in addition to the addition of resin as expressed above, I add about 0.5 per cent of a paraffin size, the percentage being by weight of solids to dry weight of fibres. This paraffin size is added simultaneously with the addition of the resin, preferably as an emul-

sion. The pH of the slurry after the addition of the resin and size is usually approximately 9.5 to 9.8. The precipitation of the resin is preferably carried out by adding a ten per cent sulfuric acid solution until a pH of 6.0 to 6.5 is reached, then adding a ten per cent alum solution until a final pH of 5.0 to 5.5 is reached, after which the board may be immediately formed. The acidification could be entirely accomplished by the use of an acid alone or an acidic salt alone, but again economy and ease of handling dictates the use of a large percentage of sulfuric acid and a final adjustment of the pH by the use of alum. Thus when the board is formed the paraffin is intimately associated throughout and aids in repelling moisture and water.

In referring to the resin as a phenolic resin I do not necessarily mean that a phenol-formaldehyde condensation product should be utilized, since various other phenols such as cresylic acid and resorcinol may be substituted for the phenol and various other aldehydes may be substituted for the formaldehyde, as is well known in the art. In referring to the condensation product as being in the B-stage or incipient C-stage, reference is made to the classification established by L. H. Baekeland in his article "The syntheses, constitution and uses of Bakelite," published in the Journal of Industrial and Engineering Chemistry, volume I, Number 3, March 1909, pages 149, 155, in which he defines three stages of phenolic resins as follows: The A-stage or initial condensation product may be liquid, viscous, pasty or solid at ordinary temperatures. It is soluble in alcohol, acetone, phenol, glycerin and similar solvents and in sodium hydroxide. Solid A is brittle and melts if heated. All variations of A heated long enough under suitable conditions will change first into B, then finally into C. B-stage, or intermediate condensation product, is solid at all temperatures. It is brittle, being slightly harder than solid A at ordinary temperatures. It is insoluble in all solvents but may swell in acetone, phenol or terpenol without entering into complete solution. When heated it does not melt, but softens and becomes elastic and rubberlike, but upon cooling again becomes hard and brittle. Further heating under suitable conditions changes it into C. Although B is infusible, it can be molded under pressure in the presence of heat to a homogeneous, coherent mass and further changed into C by the proper application of heat. C-stage or final condensation product is infusible, insoluble in all solvents, unattacked by acetone, indifferent to ordinary acids or alkaline solutions, is destroyed by boiling in concentrated sulfuric acid, but stands boiling with diluted sulfuric acid, does not soften to any serious extent if heated, stands temperatures of 300° C., and begins to be destroyed by higher temperatures and chars without entering into fusion.

I have found that any of several water-soluble, alkaline, phenolic resins in the intermediate condensation product stage, which may be purchased in open market, may be utilized to advantage in my process, such resins being in the B-stage in solution in an alkali such as sodium hydroxide, even though Baekeland's classification seems to deny solubility. I prefer the Redfern resin for its greater retention, the improved results therefrom, and its ease of handling and recapture, which resin Redfern describes as being in the incipient C-stage, meaning that he has produced a resin at the extreme limit of the B-stage which may rapidly convert to C-stage resin upon the

application of heat. When using any phenolic resin in B-stage I find that the retention thereof achieved in my process is such that the resin and other chemicals present in the fibres remain in place when heat and pressure are applied to a wet mat so that the final product is homogeneous throughout and is not surface-discolored or charred by the presence of burnt sugars or the like. The homogeneity of the final product is more pronounced with the use of Redfern resin, since the conversion of the resin into the final infusible, insoluble C-stage product is more rapidly achieved after the application of heat and pressure is begun. The Redfern resin is sold as "American-Marietta 113," and other usable resins are "Adhesive Products 3910," "Durez 11857" and "Bakelite BV 9700."

Having described the invention in particularity and in its broader aspects, I claim as my invention all such modifications thereof as may come within the true spirit and scope of the appended claims.

I claim:

1. The process of forming artificial boards and boardlike articles which comprises reducing cellulosic material to fibres, mixing the fibres with water to form a slurry, thoroughly mixing into the slurry an alkaline solution of a water-soluble, thermosetting, intermediate condensation product of a phenol-aldehyde resin in the proportion of about 3.5 per cent resin solids to fibres and about 0.5 per cent paraffin size based on the dry weight of the fibres, agitating the mixture for at least one-half hour, adding an acid in sufficient quantity substantially to neutralize the mixture in order to precipitate the resin in situ and simultaneously adding sufficient alum to coalesce the size and fibres, straining the water from the slurry to form a mat of entangled, resin-bearing, sized fibres, and compressing the mat while heating it to form a finished product of sized fibres at least partially bound together by the infusible,

insoluble, final condensation product of the resin.

2. The process of forming artificial boards and boardlike articles which comprises reducing wood or woody substances to fibres, mixing the fibres with water to form a slurry, thoroughly mixing into the slurry an alkaline, water-soluble solution of a thermosetting, intermediate condensation product of a phenol-aldehyde resin while adding a paraffin size, allowing the resin and size to remain in the slurry for a period of time in the range of twenty minutes to one hour to establish sorption of the resin solution by the fibres, mixing sufficient acid to the mixture to precipitate the resin in situ while adding sufficient alum to fix the size, straining the water from the slurry to form a mat of entangled, resin-bearing, sized fibres, and compressing the mat while heating it to form a finished product of sized fibres at least partially bound by an infusible, insoluble, final condensation product of the resin.

GORDON E. TOWER.

#### References Cited in the file of this patent

#### UNITED STATES PATENTS

| Number     | Name      | Date           |
|------------|-----------|----------------|
| Re. 23,347 | Redfern   | Mar. 20, 1951  |
| 1,160,365  | Baekeland | Nov. 16, 1915  |
| 1,684,755  | Clapp     | Sept. 18, 1928 |
| 2,027,090  | Carter    | Jan. 7, 1936   |
| 2,036,156  | Lundback  | Mar. 31, 1936  |
| 2,068,926  | Nevin     | Jan. 26, 1937  |
| 2,173,391  | Ellis     | Sept. 19, 1939 |
| 2,343,090  | Smith     | Feb. 29, 1944  |
| 2,539,183  | Child     | Jan. 23, 1951  |

#### FOREIGN PATENTS

| Number | Country       | Date                     |
|--------|---------------|--------------------------|
| 28,155 | Great Britain | June 29, 1911<br>of 1910 |

#### OTHER REFERENCES

Boehm: Paper Trade J., pp. 35-38, May 2, 1940.